# EUROPEAN PATENT SPECIFICATION

(11) **EP 1 059 362 B1**
(45) Date of publication and mention of the grant of the patent: **30.12.2009**
(21) Application number: 00202018.8
(22) Date of filing: 07.06.2000
(51) Int. Cl.: C22C 21/14, C22C 21/16, C22C 21/00

(54) **Aluminium extrusion alloy**
Aluminium-Strangpresslegierung
Alliage d'aluminium d'extrusion

(30) Priority: 11.06.1999 EP 99201855
(43) Date of publication of application: 13.12.2000
(73) Proprietor: Aleris Aluminum Koblenz GmbH, 56070 Koblenz (DE); Aleris Aluminum Duffel BVBA, 2570 Duffel (BE)
(72) Inventor: Hurd, Timothy John, 1921 CS Akersloot (NL); Vieregge, Klaus, 56237 Nauort (DE); Tack, Louis Walter Marie Paul, 2840 Reet (BE); Mulkers, Arne, 2000 Antwerpen (BE)
(74) Representative: Müller, Frank Peter

(56) References cited:
- EP-A- 0 676 480
- EP-A- 0 718 072
- GB-A- 2 318 586
- US-A- 4 589 932
- US-A- 5 342 459
- PATENT ABSTRACTS OF JAPAN vol. 1995, no. 04, 31 May 1995 (1995-05-31) -& JP 07 003409 A (FURUKAWA ELECTRIC CO LTD:THE), 6 January 1995 (1995-01-06)
- PATENT ABSTRACTS OF JAPAN vol. 1997, no. 01, 31 January 1997 (1997-01-31) -& JP 08 225874 A (FURUKAWA ELECTRIC CO LTD:THE;NISSAN MOTOR CO LTD), 3 September 1996 (1996-09-03)
- PATENT ABSTRACTS OF JAPAN vol. 1997, no. 01, 31 January 1997 (1997-01-31) -& JP 08 232035 A (SUMITOMO LIGHT METAL IND LTD), 10 September 1996 (1996-09-10)

## Description

### FIELD OF THE INVENTION

The invention relates to an aluminium extrusion alloy and extruded sections thereof, containing Mn, Mg, Cu and Si, which aluminium extrusion alloy is particular suitable for application in brazed assemblies, and further to a method of its manufacture.

### DESCRIPTION OF THE RELATED ART

In the prior art, aluminium alloys are the alloys of choice for heat exchanger applications. These alloys are selected for their desirable combination of strength, low weight, good thermal and electrical conductivity, brazeability, corrosion resistance and formability.

Typical applications include automotive heater cores, radiators, evaporators, condensers, charge air coolers, and transmission/engine oil coolers.

At present brazed heat-exchanger devices, such as for example automotive radiators, are often provided with mechanical fasteners made of extruded Aluminium Association (AA)6063-series alloy, preferably in a T8-temper. A T8-temper involves solution heat treatment of the extruded product, cold working and then artificially ageing. This application requires excellent mechanical properties and a good machinability of the extruded product for putting in a mechanical thread. Additionally at least a reasonable corrosion resistance is required. The chemical composition of standard AA6063 alloy is, in weight percent:-
Si 0.2 - 0.6
Mg 0.45 - 0.9
Fe 0.35 max.
Cu 0.1 max.
Mn 0.1 max.
Cr 0.1 max.
Zn 0.1 max.
Ti 0.1 max.
balance aluminium and inevitable impurities.
Further the AA6063 alloy is extensively used in the T6 (artificially aged) temper. When AA6063 alloy is being applied in combination with a Controlled Atmosphere Brazing (CAB) process, a brazing flux is applied to enhance the brazeabilty of the brazing alloy. A well known CAB brazing process is the Nokolok (trade name) brazing process and involves the use of a non-corrosive flux made up of a mixture of potassium and fluoroaluminates. The flux functions at brazing temperatures by melting, spreading and dissolving the oxide film. However, due to the presence of the magnesium in the AA6063 alloy the flux material tends to get poisoned by the formation of MgO, which results in a bond of poor quality. This disadvantage can only be partly be overcome by applying higher loads of brazing flux material. Another solution would be the application of mechanical fasteners made of AA3003 material since it comprises magnesium in a range of up to 0.05%. But this material is too weak to put in a thread, leading to pull out on testing. The chemical composition of standard AA3003 alloy is, in weight percent:-
Si < 0.6
Fe < 0.7
Cu 0.05 - 0.20
Mn 1.0 - 1.5
Zn 0.10
balance aluminium and inevitable impurities.

Some other disclosures of aluminium extrusion alloys found in the prior art literature will be mentioned below.

US-A-5,342,459 (Alcoa) discloses an aluminium extrusion alloy and a method of its manufacture, the alloy consisting of, in weight percent:-
Mg 0.5 - 1.3
Si 0.4 - 1.2
Cu 0.65 - 1.2
Mn 0.1 - 1.0
balance aluminium and inevitable impurities.

US-A-4,589,932 (Alcoa) discloses an aluminium extrusion alloy and a method of its manufacture, the alloy consisting of, in weight percent:-
Mg 0.5 - 1.3, preferably 0.7 - 1.2
Si 0.4 - 1.2, preferably 0.6 - 0.9
Cu 0.6 - 1.1, preferably 0.6 - 0.95
Mn 0.1 - 1.0, preferably 0.2 - 0.6
Fe < 0.6
and with the proviso that %Mg > %Si + (0.1 to 0.4)
balance aluminium and inevitable impurities.
In order to improve the machining characteristics of the alloy each of lead and bismuth in a range of 0.3 to 0.7% may be added to the alloy.

EP-A-0676480 (Northwest Aluminum) discloses two very wide groups of high strength Al-Mg-Si extrusion alloys.
The first group of aluminium alloys consists of, in weight percent:-
Si 0.2 - 2.0
Mg 0.3 - 1.7
Cu 0.32 - 1.2
Mn 0 - 1.1
Cr 0.01 - 0.4
at least one element selected from the group consisting of:-
   V 0.01 - 0.3
   Be 0.001 - 0.1
   Sr 0.01 - 0.1
balance aluminium and inevitable impurities.
The second group of aluminium alloys consists of, in weight percent:-
Si 0.6 - 1.2
Mg 1.0 - 1.6
Cu 0.4 - 1.0
Mn < 0.05
Cr 0.05 - 0.3
at least one element selected from the group consisting of:-
   V 0.01 - 0.3
   Be 0.001 - 0.05
   Sr 0.01 - 0.1
balance aluminium and inevitable impurities.
Both aluminium extrusion alloys are preferably provided in a T6-temper condition.

WO-A-99/07906 (Hoogovens) discloses an aluminium alloy for welded structures and brazing application, having the following composition in weight percent:-
Mg 0.5 - 1.5
Zn 0.1 - 3.8
Si 0.05 - 1.5
Mn 0.2 - 0.8
Zr 0.05 - 0.25
Cr < 0.3
Cu < 0.3
Fe < 0.5
Ag < 0.4
Ti < 0.2
balance aluminium and inevitable impurities.

### SUMMARY OF THE INVENTION

An object of the present invention as defined in the claims is to provide an aluminium extrusion alloy capable of obtaining post-brazing mechanical properties and corrosion resistance at least comparable to standard AA6063, and being capable of being processed in at least a Controlled Atmosphere Brazing (CAB) process.

A further object of the present invention is to provide an aluminium extrusion alloy having machinability characteristics at least equal to standard AA6063 extruded products, typically in a T8-temper.

Another object of the present invention is to provide a method of manufacturing extruded sections of the new aluminium alloy.

And another object of the present inventions is to provide a method of manufacturing an assembly of brazing components, wherein one of the components is made from the aluminium extrusion alloy of the invention.

According to the invention in one aspect there is provided an aluminium extrusion alloy having the following composition in weight percent:-
Mn 1.0 - 1.4
Cu 0.2 - 2.0
Mg 0.1 - 0.6
Si 0.15 - 1.0
Fe 0.8 max.
Zn 0.25 max.
Ti 0.15 max.
Cr 0.35 max.
Zr and/or V in total 0.35 max.
others up to 0.05 each, total 0.15
balance Al, and with the proviso that (Cu+Mg)> 0.7.

In this way it is achieved that the aluminium extrusion alloy of the invention has similar post-braze mechanical strength as compared to AA6063 in the same temper and better than AA3003 material, a corrosion resistance as tested in a SWAAT test environment equivalent to AA6063 material in the same temper, and further the machinability characteristics of the present extrusion alloy are equal to or better than AA6063 material in the same temper and better than AA3003 material. Further the aluminium extrusion alloy of the invention can be used to manufacture devices via a brazing process, and in particular in a Controlled Atmosphere Brazing process.

It should be mentioned here that the aluminium alloy composition range is known from EP-A-0718072, in which document it is mentioned that the alloy is used as a rolled product only as core alloy for brazing sheet having on at least one side thereof a brazing layer of an aluminium alloy containing silicon as main alloying element.

The reasons for the limitations of the alloying elements of the aluminium extrusion alloy according to the invention are described below. All compositions are by weight.

Mn is an important alloying element in the alloy according to the invention. And should be in the range of 1.0 to 1.4%. Below 1.0% there is not a sufficient effect, and above 1.4% it may result in the formation of detrimental large intermetallic particles. In this range the Mn present allows for a solid solution hardening effect because sufficient Mn is retained in solid solution for the desired increase in strength.

Cu is one of the main alloying elements in order to obtain the desired strength level, in particular by means of solution hardening. At least 0.2% is required for obtaining the desired strength and corrosion resistance, while a Cu content of over 2.0% does not produce any significant improvements in respect of strength, and may further result in the formation of detrimental low-melting eutectics. A more preferred lower limit for the Cu level is 0.5%. A more preferred Cu content is in a range of 0.65 to 1.5% in order to achieve an optimisation in the desired properties. A very suitable range for the Cu-content is 0.65 to 0.9% as a compromise in mechanical strength after extrusion, mechanical strength in the post-braze condition, post-braze corrosion resistance and extrudability.

Mg is another main alloying elements in combination with the Cu and Si present in order to obtain the desired properties. The Mg can be present in the range of 0.1 to 0.6%. In case the extrusion alloy is used for application in a Controlled Atmosphere Brazing process a more suitable Mg-content is in the range of 0.1 to 0.35%. In case the extrusion alloy is used for application in a vacuum brazing process a suitable Mg-content is in the range of 0.3 to 0.6%.

For strength and corrosion resistance preferably the proviso (Cu+Mg)>1.0 is met. Thereby a good corrosion resistance of a product manufactured via a brazing process is obtained.

Si is another important alloying element in the aluminium alloy according to this invention. The main reason is to enable the formation of Mg₂Si precipitation required to improve the strength by means of ageing before and after brazing. Further, the addition of Si results in an increased solution hardening of the alloy after brazing. Below 0.15% there is no effect of the Si, and above 1.0% it may result in the formation of detrimental low-melting eutectics and also in the formation of large intermetallic particles. A more suitable minimum level of Si is 0.20%, more preferably of 0.30%, and most preferably of 0.40%. A more suitable maximum level of Si is 0.70%, and more preferably 0.60% as a compromise in extrudability, tensile strength and corrosion resistance.

Fe is a known impurity element in this type of aluminium alloys. Its presence should be limited to a maximum of 0.8%, and preferably to a maximum of 0.4%, in order to optimise the mechanical properties and extrudability.

Zn is considered to be an impurity element also and can be tolerated up to 0.25%, but is preferably less than 0.15%, and more preferably less than 0.10%.

Ti is important as a grain refiner during solidification of cast extrusion billets or ingots. The preferred range of Ti is not more than 0.15%, but preferably is less than 0.10%, and more preferably is less than 0.05%.

Cr improves the corrosion resistance of the alloy. However, Cr limits the solubility of Mn and further reduces the extrudability of the aluminium alloy. Therefor, to avoid formation of coarse primaries and to improve extrusion capability, the Cr content must not be more than 0.35%, preferably not more than 0.2%, and more preferably less than 0.05%.

The optionally added Zr and/or V improves amongst other things the strength of the aluminium extrusion alloy. A more preferred maximum for these elements alone or in combination is 0.25%. A more suitable level of these elements alone or in combination is in the range of 0.05 to 0.25%.

Although Cr, Zr and V can de added in the given ranges to control extrudability and mechanical properties, in a preferred embodiment of the aluminium extrusion alloy according to the invention, each of Cr, Zr and V are at impurity level, meaning below 0.05%, in order to control the costs of the aluminium alloy and to increase its recycleability.

The balance is aluminium and inevitable impurities. Typically each impurity element is present at 0.05% maximum, and the total of impurities is 0.15% maximum.

The invention is further embodied in an extruded section having a composition of the aluminium alloy of this invention as set out above. The extruded section can be provided at least in any one of a number of tempers selected from the following types T3, T4, T6, T8 and T9, or modifications thereof.

The invention also provides in a method of manufacturing an extruded section comprising the aluminium extrusion alloy set out above, which method comprises the following sequential steps:-
(a) casting the aluminium alloy into ingots;
(b) preheating the cast ingot;
(c) hot extrusion of the preheated cast ingot into an extruded product;
(d) rapid cooling of the extruded product to below 150°C;
(e) ageing of the product.

In this way a method is provided which allows for the production of extruded sections capable of obtaining similar post-braze mechanical strength as compared to AA6063 in the same temper and better than AA3003 material, a corrosion resistance as tested in a SWAAT test environment equivalent to AA6063 material in the same temper, and further to obtain machinability characteristics equal to or better than AA6063 material in the same temper and better than AA3003 material. Further the aluminium extrusion alloy obtained by the method according to the invention can be used to manufacture devices via various brazing processes, and in particular in a Controlled Atmosphere Brazing process.

For casting the inventive aluminium alloy into ingots or extrusion billets in any diameter both continuous and semi-continuous casting processes can be used. Different configurations of castings can also be used to produce the desired extrusion shape.

After casting, the aluminium alloy may be homogenised. The aim of the homogenising treatment is amongst other things, to homogenise the microstructure, to dissolve the relevant elements or components such as Mg₂Si, to level off possible residual stresses resulting from the casting process, and to spheroidize sharp or needle shaped intermetallic compounds formed during solidification of the aluminium alloy. A homogenisation treatment in the temperature range of 560 to 610 °C for a soaking time in the range of 5 to 24 hours results in the optimised properties. A longer homogenisation time is not disadvantageous, but is not required and only serves to raise the costs of production. Alternatively the homogenisation treatment may be omitted. Omitting the homogenisation treatment still allows for very good extrusion characteristics, and resulting in a final extruded product having an improved post-braze mechanical properties while the corrosion resistance is somewhat reduced.

After casting or following homogenisation treatment, the cast billets are preheated at temperatures between 500 and 540°C.

Subsequently, the ingot or extrusion billet is processed into products via a hot extrusion process, wherein either direct or indirect extrusion techniques may be used. The ingot temperature during extrusion is preferably in the range of 500 to 540°C. Using a hot extrusion process the aluminium alloy in accordance with the invention can be processed in both solid and hollow extruded sections. In this temperature range it has been found that the alloy in accordance with the invention has a high extrudability, and very similar to AA6063 alloys.

It should be understood that the aluminium extrusion alloy in accordance with the invention can be extruded in any configuration including channels, bars, seat rails, I-beams, angles, tubing, heat exchanger tubing, architectural shapes, rectangular hollows, rods, or other complex extruded shapes.

After extrusion, the alloy of the invention should be rapid cooled to below 150°C by means of water or water spray in order to prevent or minimise uncontrolled precipitation. This is also designated by the term "press-quenching". Following cooling to below 150°C, the extruded section is further cooled to about room temperature.

In a following step, the extruded product is aged to the desired level of mechanical and physical properties. The ageing may be natural ageing (at ambient temperature) and/or artificial ageing at an elevated temperature, preferably in the range of 100 to 250°C. A natural ageing period of 3 months is typical for this. Artificial ageing can result in an 0.2% yield strength of 270 MPa or more. Preferably the artificial ageing is executed for a time period in the range of 1 to 100 hours. For example, the artificial ageing is executed at about 160°C for a time period in the range of 3 to 100 hours, preferably for a time period in the range of 3 to 15 hours, or at an equivalent combination of time and temperature giving a similar ageing effect.

In order to further improve the mechanical properties the extruded product is cold worked after extrusion. The cold working may be performed prior to or after the ageing treatment, but there is a preference for cold working prior to the ageing treatment. The product may be cold worked, for example, by drawing or stretching up in the range of 4 to 20% of its original length. Preferably, the cold reduction is in the range of 5 to 18% of its original length to optimise properties.

The extruded section can be provided in at least any one of the following tempers selected from the group of T3 (solution heat treated, cold worked, and naturally aged to a substantially stable condition), T4 (solution heat treated and naturally aged to a substantially stable condition), T6 (solution heat treated and then artificially aged), T8 (solution heat treated, cold worked, and then artificially aged), T9 (solution heat treated, artificially aged, and then cold worked), and modifications thereof.

By artificial ageing treatment the extruded section is capable of obtaining an 0.2% yield strength of at least 270 MPa or more, and preferably of 280 MPa or more. Further, by artificial ageing treatment the extruded section is capable of obtaining an ultimate tensile strength of 290 MPa or more, preferably of 310 MPa or more, and in the best examples of 325 MPa or more.

In a further embodiment of the method in accordance with the invention the extruded and aged section may be worked into a more suitable shape, for example by means of machining. The worked product may be added to an assembled device, for example an automotive radiator, which device is subsequently joined in a brazing process. Following the brazing cycle the brazed assembly together with the worked product is cooled to below 100°C and preferably to room temperature by a set cooling rate. Following cooling to room temperature the brazed assembly is allowed to age to final desired mechanical properties. The extrusion alloy of the invention is capable of obtaining a post-braze 0.2% yield strength of at least 100 MPa or more, preferably of 120 MPa or more, and in the best examples of 140 MPa or more, and a post-braze ultimate tensile strength of at least 200 MPa or more, and preferably of 220 MPa or more, by means of natural ageing at ambient temperatures. If desired the extrusion alloy in accordance with the invention is capable of reaching even higher mechanical properties when artificially aged.

An advantage of the application of the extrusion alloy in accordance with the present invention is that it provides high mechanical properties both before and after a brazing cycle. The mechanical properties are at least similar to AA6063 material in the same temper, while the inventive alloy further allows for a favourable processing in a CAB brazing process.

In another aspect of the invention there is provided a method of manufacturing an assembly of brazed components, comprising the steps of:-
(a) forming said components of which at least one is made from an aluminium extrusion alloy as set out above or the extruded section obtained from the method as set out above;
(b) assembling the components into an assembly;
(c) brazing the assembly at elevated temperature for a period long enough for melting and spreading of the filler material;
(d) cooling the brazed assembly to below 100°C;
(e) ageing of the brazed and cooled assembly to achieve an 0.2% yield strength of at least 100 MPa, and preferably of at least 120 MPa, and more preferably of at least 140 MPa or more.

In accordance with the invention it has been found that the cooling rate after the brazing cycle plays a role in obtaining the desired strength level of the brazed assembly. The cooling rate should not be below 30°C/min. More preferably the cooling rate after brazing is at least 50°C/min, and more preferably at least 60°C/min, and most preferably at least 70°C/min. Increasing the cooling rate after the brazing cycle can give rise to a further increase in the obtainable strength levels. Surprisingly it has been found that extruded sections having a composition in accordance with the invention as set out above and which have been homogenised during their manufacture from a cast ingot into extruded sections respond to the influence of the cooling rate after brazing. Whereas the extruded sections having a composition in accordance with the invention as set out above and which have not been homogenised during their manufacture from a cast ingot into extruded sections respond to a much lesser extend on the cooling rate after brazing and the subsequent ageing.

In a preferred embodiment of the method during the brazing step (c) a controlled atmosphere (CAB) is being used whereby a suitable brazing flux material is used.

In another aspect of the invention there is provided a brazed assembly comprising at least one member being an extruded section comprising the aluminium alloy of the invention, and having a post-braze 0.2% yield strength of at least 100 MPa or more, preferably of at least 120 MPa or more, and more preferably of at least 140 MPa or more.

### EXAMPLES

The aluminium extrusion alloy and the method of its manufacture in accordance with the invention will now be illustrated by non-limitative examples.

### Example 1.

On an industrial scale of testing four alloys composition in accordance with the invention, see Table 1, have been DC-cast into 300 diameter billets. Three have been homogenised for 8 hours at 600°C, and one has not been homogenised. Sequentially all billets have been preheated to about 500°C and then extruded at about 520°C into rods of 30mm or 15mm diameter, then press quenched to below 150°C, cooled to room temperature, cold worked for various cold working degrees and artificial aged to T8-temper by holding for 10 hours at 160°C. In Table 2 an overview is given of the processing parameters applied.

The extruded rods have been tested for their mechanical properties, 0.2% yield strength (0.2% YS), ultimate tensile strength (UTS) and elongation at fracture (A₅₀), see Table 2, and for their machinability characteristics. Table 3 shows typical properties of AA6063-T8 and AA3003-H111 extruded material.

The machinability characteristics of the alloy of the invention is similar to or better than AA6063 material in the same T8-temper; both give about 1 cm long, spiral or curly chips. The machinability is much better than AA3003 material, which gives unbroken chips being arranged around the cutting tools. Further it is believed that from a machinability point of view a T9-temper provides better results than T8-temper material, resulting in shorter chips and the cut surface is more shiny and more smooth.

From Table 2 and 3 it can be seen that the alloy of the invention is capable of obtaining similar or better mechanical properties than AA6063 material, both alloys being in a T8-temper. Further it can be seen that non-homogenised material has mechanical properties in the same range as homogenised material. The alloy of the invention is capable of obtaining mechanical properties significantly better than AA3003-H111 material, which material would be the normal alternative for AA6063 when further processed in a CAB brazing process.

**Table 1. Alloy composition in weight %.**

| **Alloy** | **Si** | **Fe** | **Cu** | **Mn** | **Mg** | **Balance** |
|---|---|---|---|---|---|---|
| **1** | 0.47 | 0.23 | 0.73 | 1.14 | 0.31 | Al + impurities |
| **2** | 0.45 | 0.29 | 0.81 | 1.17 | 0.30 | Al + impurities |
| **3** | 0.5 | 0.23 | 0.70 | 1.25 | 0.29 | Al + impurities |
| **4** | 0.46 | 0.21 | 0.74 | 1.09 | 0.30 | Al + impurities |

**Table 2. Processing parameters and mechanical properties in a T8-temper.**

| | **Alloy 1** | **Alloy 2** | **Alloy 3** | **Alloy 4** |
|---|---|---|---|---|
| **Homogenisation [T/t]** | 600°C/8h. | 600°C/8h. | no | 600°C/8h. |
| **Press speed [m/min]** | 5 | 5 | 5 | 5 |
| **Extrusion ratio** | 17.2 | 20.8 | 17.2 | 17.2 |
| **Diameter rod [mm]** | 30 | 15 | 30 | 30 |
| **Press quench** | yes | yes | yes | yes |
| **Cold Reduction [%]** | 14 | 17 | 14 | 18 |
| **Ageing [T/t]** | 160°C/10h. | 160°C/10h. | 160°C/10h. | 160°C/10h. |

| **Mechanical properties** | | | | |
|---|---|---|---|---|
| **0.2% YS [MPa]** | 282 | 286 | 290 | 304 |
| **UTS [MPa]** | 313 | 325 | 326 | 332 |
| **A₅₀ [%]** | 10 | 12 | 12 | 10 |
| **Hardness [HB]** | 84 | 83 | 84 | 85 |

**Table 3. Comparable extruded material.**

| **Property** | **AA6063-T8** | **AA3003-H111** |
|---|---|---|
| **0.2% YS [MPa]** | 270 | 70 |
| **UTS [MPa]** | 290 | 135 |
| **A₅₀ [%]** | 15 | 35 |
| **Hardness [HB]** | 80 | 40 |

### Example 2.

The alloys as manufactured in Example 1 will usually be provided to customers in the aged condition for further application. In case the material is used to manufacture a brazed assembly, the material is preferably in a T8- or T9-temper. When used in manufacturing a brazed assembly, the alloy of the invention will be subjected to a heat-treatment in accordance to the braze cycle, which affects its mechanical properties. In order to investigate this influence extruded material of alloys 2, 3 and 4 of example 1 in the T8-temper has been subjected to a simulated braze cycle, where the material is heated up to 538°C in 10 min., then further heated from 538 to 591°C in 6 min, a dwell time of 3 min at 591°C, and then cooled with variable cooling rates.

Following cooling the material has been natural aged and tested for its mechanical properties, average over two samples tested. Also AA6063 material has been subjected to this simulated braze cycle, and tested. The results of the mechanical properties are listed in Table 4. The post-braze 0.2% yield strength (PS), ultimate tensile strength (UTS), and elongation (Elong.) of AA3003 material is typically in the range of 30 to 40 MPa, 95 to140 MPa, and 28% respectively. Following brazing the material has also been tested for 15 days in a SWAAT test environment, which is equivalent to long life properties for sheet material.

From the results of Table 4 it can be seen that the alloy of the invention has significant higher post-braze mechanical properties than AA3003-material. Further it can be seen that that for homogenised material the mechanical properties tend to increase with increasing cooling rate after brazing. However, non-homogenised material (Alloy 3 material) shows almost no influence of the cooling rate after brazing on the post-braze mechanical properties. Further, the non-homogenised material has significantly higher strength and lower elongation directly after brazing and shows almost no influence of natural ageing time. The results with respect to the non-homogenised material were unexpected and can not readily be explained. The alloy of the invention is capable of obtaining mechanical properties at least similar to AA6063 material.

After 15 days in a SWAAT test, the AA6063 material showed a shiny bright surface with only slight pitting with a PA qualification. Alloy 2 material showed also a shiny bright surface with somewhat deeper pits with a PA qualification. The alloy 4 material showed uniform attack and was given a PB qualification. The alloy 3 materials showed a uniform attack, and was given a PB/C qualification. From these results it can be concluded that the alloy in accordance with the invention is capable of obtaining an equivalent corrosion resistance as AA6063 material.

**Table 4. Post-braze mechanical properties as function of alloy composition, days of natural ageing after brazing and cooling rate after the braze cycle.**

| | **5 days natural ageing** | | | **30 days natural ageing** | | |
|---|---|---|---|---|---|---|
| **Material** | **PS** **[MPa]** | **UTS.** **[MPa]** | **Elong.** **[%]** | **PS** **[MPa]** | **UTS** **[MPa]** | **Elong.** **[%]** |
| **Alloy 2 - 15 mm rod** | | | | | | |
| 50 °C/min | 153 | 225 | 15 | 159 | 232 | 19 |
| 70 °C/min | 161 | 235 | 18 | 157 | 231 | 17 |
| **Alloy 3 - 30 mm rod (non-homogenised)** | | | | | | |
| 30 °C/min | 165 | 239 | 9 | 163 | 237 | 16 |
| 50 °C/min | 166 | 238 | 8 | 167 | 238 | 15 |
| 70 °C/min | 169 | 238 | 8 | 166 | 238 | 15 |
| **Alloy 4 - 30 mm rod** | | | | | | |
| 50 °C/min | 96 | 143 | 18 | 95 | 135 | 19 |
| 70 °C/min | 103 | 148 | 16 | 98 | 151 | 19 |
| **AA6063 - 30 mm rod** | | | | | | |
| 50 °C/min | 92 | 143 | 21 | 108 | 148 | 21 |
| 60 °C/min | 93 | 141 | 23 | 107 | 152 | 19 |
| 70 °C/min | 102 | 158 | 23 | 110 | 181 | 20 |

## Claims

1. A method of manufacturing an extruded section of an aluminium extrusion alloy, which method comprises the sequential steps of:-
(a) casting the alloy into ingots having a composition in weight%:
Mn 1.0 - 1.4
Cu 0.2 - 2.0
Mg 0.1 - 0.6
Si 0.15 - 1.0
Fe 0.8 max.
Zn 0.25 max.
Ti 0.15 max.
Cr 0.35 max.
Zr and/or V in total 0.25 max.
others up to 0.05 each, total 0.15
balance aluminium,
and with the proviso that (Cu+Mg)>0.7, and preferably (Cu+Mg)>1.0,
(b) preheating the cast ingot;
(c) hot extrusion of the preheated cast ingot into an extruded product;
(d) rapid cooling of the extruded product to below 150°C by means of water or water spray;
(e) ageing of the extruded and cooled product to achieve an 0.2% yield strength of at least 270 MPa.

2. The method according to claim 1, wherein the method further comprises prior to step (b) the step of homogenising the cast ingot in a temperature range of 560 to 610°C for a soaking time in the range of 5 to 24 hours.

3. The method according to claim 1 or 2, wherein the hot extrusion during step (c) is carried out with an extrusion billet in a temperature range of 500 to 540°C.

4. The method according to any one of claims 1 to 3, wherein the alloy has a Cu-content in the range of 0.65 - 2.0%, and preferably 0.65 - 0.90%.

5. The method according to any one of claims 1 to 4, wherein the alloy has Si-content in the range of 0.30 - 1.0%, and preferably 0.4 - 1.0%.

6. The method according to any one of claims 1 to 5, wherein the alloy has Mg-content in the range of 0.1 - 0.35%.

7. The method according to any one of claims 1 to 6, ,wherein the alloy has Mg-content in the range of 0.3 - 0.6%.

8. The method according to any one of claims 1 to 7, wherein the extruded section made of the aluminium extrusion alloy is provided in a T8 or in a T9 condition

9. Method of manufacturing an assembly of brazed components, comprising the steps of:-
(a) forming said components of which at least one is made from an aluminium extrusion alloy having a composition in weight%: Mn 1.0 - 1.4, Cu 0.2 - 2.0, Mg 0.1 - 0.6, Si 0.15 - 1.0, Fe 0.8 max., Zn 0.25 max., Ti 0.15 max., Cr 0.35 max., Zr and/or V in total 0.25 max., others up to 0.05 each, total 0.15, balance aluminium, and with the proviso that (Cu+Mg) >0. 7, and preferably (Cu+Mg)>1.0,, obtained from the method in accordance with any one of claims 1 to 8;
(b) assembling the components into an assembly;
(c) brazing the assembly at elevated temperature for a period long enough for melting and spreading of the filler material;
(d) cooling the brazed assembly to below 100°C;
(e) ageing of the brazed and cooled assembly to achieve an 0.2% yield strength of at least 100 MPa, and preferably of at least 120 MPa.

10. Method according to claim 9, wherein the brazing step (c) further comprises using a brazing flux and a controlled atmosphere (CAB).

11. Method according to claim 9 or 10, wherein during step (d) the brazed assembly is cooled below 100°C with a cooling rate of at least 50°C/min.

12. Method according to any one of claims 9 to 11, wherein the aluminium extrusion alloy has a Cu-content in the range of 0.65 - 2.0%, and preferably 0.65 - 0.90%.

13. Method according to any one of claims 9 to 12, wherein the aluminium extrusion alloy has a Si-content in the range of 0.30 - 1.0%, and preferably 0.4 - 1.0%.

14. Method according to any one of claims 9 to 13, wherein the aluminium extrusion alloy has a Mg-content in the range of 0.1 - 0.35%.

15. Method according to any one of claims 9 to 14, wherein the aluminium extrusion alloy has a Mg-content in the range of 0.3 - 0.6%.

16. Brazed assembly comprising at least one member comprising an extruded section having a composition in weight%: Mn 1.0 - 1.4, Cu 0.2 - 2.0, Mg 0.1 - 0.6, Si 0.15 - 1.0, Fe 0.8 max., Zn 0.25 max., Ti 0.15 max., Cr 0.35 max., Zr and/or V in total 0.25 max., others up to 0.05 each, total 0.15, balance aluminium, and with the proviso that (Cu+Mg)>0.7, and preferably (Cu+Mg)>1.0, and wherein said member has a post-braze 0.2% yield strength of at least 100 MPa, and preferably of at least 120 MPa.

## Patentansprüche

1. Verfahren zur Herstellung eines stranggepressten bzw. extrudierten Teils einer Aluminiumextrusions- bzw. -strangpresslegierung, wobei das Verfahren die aufeinanderfolgenden Schritte umfasst:
(a) Gießen der Legierung zu Barren, die eine Zusammensetzung, in Gew.-%, aufweisen von:
Mn 1.0 - 1.4
Cu 0.2 - 2.0
Mg 0.1 - 0.6
Si 0.15 - 1.0
Fe max. 0,8
Zn max. 0,25
Ti max. 0,15
Cr max. 0,35
Zr und/oder V insgesamt max. 0.25
andere jeweils bis 0,05, insgesamt 0,15 Rest Aluminium,
und mit der Maßgabe, dass (Cu+Mg) > 0,7 und bevorzugt
(Cu+Mg) > 1,0 ist,
(b) Vorwärmen des Gussbarrens,
(c) Warmextrudieren des vorgewärmten Gussbarrens in ein extrudiertes Produkt,
(d) rasches (Ab)Kühlen des extrudierten Produkts auf unter 150°C mithilfe von Wasser oder Wassersprühen,
(e) Altern des extrudierten und gekühlten Produkts, um eine 0,2-Prozent-Dehnfestigkeit von wenigstens 270 MPa zu erzielen.

2. Verfahren nach Anspruch 1, wobei das Verfahren ferner vor Schritt (b) den Schritt des Homogenisierens des Gussbarrens in einem Temperaturbereich von 560 bis 610°C für eine Durchwärmzeit im Bereich von 5 bis 24 Stunden umfasst.

3. Verfahren nach Anspruch 1 oder 2, wobei das Warmextrudieren während Schritt (c) mit einem Extrusionsknüppel in einem Temperaturbereich von 500 bis 540°C durchgeführt wird.

4. Verfahren nach einem der Ansprüche 1 bis 3, wobei die Legierung einen Cu-Gehalt im Bereich von 0,65 bis 2,0% und bevorzugt 0,65 bis 0,90% aufweist.

5. Verfahren nach einem der Ansprüche 1 bis 4, wobei die Legierung einen Si-Gehalt im Bereich von 0,30 bis 1,0% und bevorzugt 0,4 bis 1,0% aufweist.

6. Verfahren nach einem der Ansprüche 1 bis 5, wobei die Legierung einen Mg-Gehalt im Bereich von 0,1 bis 0,35% aufweist.

7. Verfahren nach einem der Ansprüche 1 bis 6, wobei die Legierung einen Mg-Gehalt im Bereich von 0,3 bis 0,6% aufweist.

8. Verfahren nach einem der Ansprüche 1 bis 7, wobei der extrudierte, aus der Aluminiumextrusionslegierung hergestellte Teil in einem T8 oder T9 Zustand bereitgestellt wird.

9. Verfahren zur Herstellung einer Anordnung aus hartgelöteten Bauteilen, umfassend die Schritte:
(a) Bilden der Bauteile, von denen wenigstens eines aus einer Aluminiumextrusionslegierung hergestellt ist, die eine Zusammensetzung, in Gew.-%, aufweist von: Mn 1,0 bis 1,4, Cu 0,2 bis 2,0, Mg 0,1 bis 0,6, Si 0,15 bis 1,0, Fe max. 0,8, Zn max. 0,25, Ti max. 0,15, Cr max. 0,35, Zr und/oder V insgesamt max. 0,25, andere jeweils bis zu 0,05, insgesamt 0,15, Rest Aluminium, und mit der Maßgabe, dass (Cu+Mg) > 0,7 und bevorzugt (Cu+Mg) > 1,0 ist, erzielt durch das Verfahren gemäß einem der Ansprüche 1 bis 8,
(b) Zusammensetzen der Bauteile zu einer Anordnung,
(c) Hartlöten der Anordnung bei erhöhter Temperatur für einen Zeitraum, der zum Schmelzen und Verteilen des Hartlots ausreicht,
(d) (Ab)Kühlen der hartgelöteten Anordnung auf unter 100°C,
(e) Altern der hartgelöteten und gekühlten Anordnung, um eine 0,2-Prozent-Dehnfestigkeit von wenigstens 100 MPa und bevorzugt wenigstens 120 MPa zu erzielen.

10. Verfahren nach Anspruch 9, wobei der Hartlötschritt (c) ferner die Verwendung eines Hartlötflussmittels und einer Schutzatmosphäre bzw. kontrollierter Atmosphäre (CAB) umfasst.

11. Verfahren nach Anspruch 9 oder 10, wobei während Schritt (d) die hartgelötete Anordnung unter 100°C mit einer Kühlgeschwindigkeit von wenigstens 50°C/min (ab)gekühlt wird.

12. Verfahren nach einem der Ansprüche 9 bis 11, wobei die Aluminiumextrusionslegierung einen Cu-Gehalt im Bereich von 0,65 bis 2,0% und bevorzugt 0,65 bis 0,90% aufweist.

13. Verfahren nach einem der Ansprüche 9 bis 12, wobei die Aluminiumextrusionslegierung einen Si-Gehalt im Bereich von 0,30 bis 1,0% und bevorzugt 0,4 bis 1,0% aufweist.

14. Verfahren nach einem der Ansprüche 9 bis 13, wobei die Aluminiumextrusionslegierung einen Mg-Gehalt im Bereich von 0,1 bis 0,35% aufweist.

15. Verfahren nach einem der Ansprüche 9 bis 14, wobei die Aluminiumextrusionslegierung einen Mg-Gehalt im Bereich von 0,3 bis 0,6% aufweist.

16. Hartgelötete Anordnung, umfassend wenigstens ein Element mit einem extrudierten Teil, der die folgende Zusammensetzung, in Gew.-%, hat: Mn 1,0 bis 1,4, Cu 0,2 bis 2,0, Mg 0,1 bis 0,6, Si 0,15 bis 1,0, Fe max. 0,8, Zn max. 0,25, Ti max. 0,15, Cr max. 0,35, Zr und/oder V insgesamt max. 0,25, andere jeweils bis 0,05, insgesamt 0,15, Rest Aluminium, und mit der Maßgabe, dass (Cu+Mg) > 0,7 und bevorzugt (Cu+Mg) > 1,0 ist, und wobei dieses Element eine 0,2-Prozent-Dehnfestigkeit nach dem Hartlöten von wenigstens 100 MPa und bevorzugt von wenigstens 120 MPa aufweist.

## Revendications

1. Procédé de fabrication d'un profilé extrudé d'un alliage d'aluminium pour extrusion, ledit procédé comprenant les étapes séquentielles consistant à :
(a) couler l'alliage en lingots ayant une composition en pourcentage en poids :
Mn 1,0 à 1,4
Cu 0,2 à 2,0
Mg 0,1 à 0,6
Si 0,15 à 1,0
Fe maximum 0,8
Zn maximum 0,25
Ti maximum 0,15
Cr maximum 0,35
Zr et/ou V au total au maximum 0,25
autres éléments présents chacun jusqu'à 0,05, pour un total de 0,15
le reste étant de l'aluminium, et avec la condition que (Cu + Mg) > 0,7, et de préférence (Cu + Mg) > 1,0,
(b) préchauffer le lingot coulé ;
(c) extruder à chaud le lingot coulé préchauffé pour donner un produit extrudé ;
(d) refroidir rapidement le produit extrudé jusqu'à une température au-dessous de 150°C au moyen d'eau ou d'eau pulvérisée ;
(e) faire recuire le produit extrudé et refroidi pour atteindre une résistance de rupture de 0,2 % d'au moins 270 MPa.

2. Procédé selon la revendication 1, dans lequel le procédé comprend en outre, avant l'étape (b), l'étape consistant à homogénéiser le lingot coulé dans une plage de température de 560 à 610°C pendant un temps de séjour dans une plage de 5 à 24 heures.

3. Procédé selon la revendication 1 ou 2, dans lequel l'extrusion à chaud pendant l'étape (c) est effectuée avec une billette d'extrusion dans une plage de température de 500 à 540°C.

4. Procédé selon l'une quelconque des revendications 1 à 3, dans lequel l'alliage présente une teneur en Cu dans la plage de 0,65 à 2,0 %, et de préférence de 0,65 à 0,90 %.

5. Procédé selon l'une quelconque des revendications 1 à 4, dans lequel l'alliage présente une teneur en Si dans la plage de 0,30 à 1,0 %, et de préférence 0,4 à 1,0 %.

6. Procédé selon l'une quelconque des revendications 1 à 5, dans lequel l'alliage présente une teneur en Mg dans la plage de 0,1 à 0,35 %.

7. Procédé selon l'une quelconque des revendications 1 à 6, dans lequel l'alliage présente une teneur en Mg dans la plage de 0,3 à 0,6 %.

8. Procédé selon l'une quelconque des revendications 1 à 7, dans lequel le profilé extrudé réalisé avec l'alliage d'aluminium pour extrusion est fourni dans une condition T8 ou dans une condition T9.

9. Procédé de fabrication d'un assemblage de composants brasés, comprenant les étapes consistant à :
(a) former lesdits composants, dont l'un au moins est réalisé à partir d'un alliage d'aluminium pour extrusion ayant une composition, en pourcentage en poids :
Mn 1,0 à 1,4, Cu 0,2 à 2,0, Mg 0,1 à 0,6, Si 0,15 à 1,0, Fe maximum 0,8, Zn maximum 0,25, Ti maximum 0,15, Cr maximum 0,35, Zr et/ou V au total au maximum 0,25, d'autres éléments allant jusqu'à 0,05 chacun avec un total de 0,15, le reste étant de l'aluminium, et avec pour condition que (Cu +Mg) > 0,7, et de préférence (Cu +Mg) > 1,0, obtenu par le procédé selon l'une quelconque des revendications 1 à 8 ;
(b) assembler les composants pour former un assemblage ;
(c) braser l'assemblage à température élevée pendant une période suffisamment longue pour amener le matériau de remplissage à fondre et à s'étaler ;
(d) refroidir l'assemblage brasé jusqu'à au-dessous de 100°C ;
(e) faire recuire l'assemblage brasé et refroidi pour obtenir une résistance à la rupture de 0,2 % d'au moins 100 MPa, et de préférence d'au moins 120 MPa.

10. Procédé selon la revendication 9, dans lequel l'étape de brasage (C) comprend en outre d'utiliser un flux de brasage et une atmosphère contrôlée (CAB).

11. Procédé selon la revendication 9 ou 10, dans lequel, pendant l'étape (d), l'assemblage brasé est refroidi jusqu'à au-dessous de 100°C avec une vitesse de refroidissement d'au moins 50°C/minute.

12. Procédé selon l'une quelconque des revendications 9 à 11, dans lequel l'alliage d'aluminium pour extrusion présente une teneur en Cu dans la plage de 0,65 à 2,0 %, et de préférence de 0,65 à 0,90 %.

13. Procédé selon l'une quelconque des revendications 9 à 12, dans lequel l'alliage d'aluminium pour extrusion présente une teneur en Si dans la plage de 0,30 à 1,0 %, et de préférence 0,4 à 1,0 %.

14. Procédé selon l'une quelconque des revendications 9 à 13, dans lequel l'alliage d'aluminium pour extrusion présente une teneur en Mg dans la plage de 0,1 à 0,35 %.

15. Procédé selon l'une quelconque des revendications 9 à 14, dans lequel l'alliage d'aluminium pour extrusion présente une teneur en Mg dans la plage de 0,3 à 0,6 %.

16. Assemblage brasé comprenant au moins un élément comprenant un tronçon extrudé ayant une composition, en pourcentage en poids : Mn 1,0 à 1,4, Cu 0,2 à 2,0, Mg 0,1 à 0,6, Si 0,15 à 1,0, Fe maximum 0,8, Zn maximum 0,25, Ti maximum 0,15, Cr maximum 0,35, Zr et/ou V au total de 0,25 au maximum, les autres allant chacun jusqu'à 0,05 et au total 0,15, le reste étant de l'aluminium, et avec pour condition que (Cu + Mg) > 0,7, et de préférence (Cu + Mg) > 1,0, et dans lequel ledit élément présente une résistance à la rupture à 0,2 % après brasage qui est d'au moins 100 MPa, et de préférence au moins 120 MPa.
